

1

2,916,374

## METHOD OF PRODUCING MULTIVALENT METAL

Robert E. Hulse, Darien, Conn., assignor to National Distillers and Chemical Corporation, New York, N.Y., a corporation of Virginia

No Drawing. Application March 13, 1957  
Serial No. 645,670

7 Claims. (Cl. 75—84.5)

This invention relates to a new and useful process for the manufacture of metal sponge. More particularly, the invention pertains to the production of zirconium sponge from zirconium tetrahalide.

The preparation of metals by reduction of their halides with stoichiometric amounts of reducing agents such as alkali metals is well known in the prior art. In an effort to avoid certain operational difficulties of the prior art processes, it has been recently proposed that metals such as zirconium may readily be prepared by first partially reducing the metal halides with an alkali metal under carefully controlled conditions to obtain a free flowing, finely divided solid, dry mixture of metal subhalide-alkali metal halide complexes. The resulting reaction mixture is then further reacted with additional alkali metal to complete the reduction to the metal in a combined reduction and sintering operation. The metal produced by following the aforescribed process while meeting most specifications often has an unduly high halogen ion content.

In accordance with the present invention, it has now been found that an excellent metal product having a halogen ion content of less than about 0.2% can be obtained directly from the metal subhalide-alkali metal halide complex mixture. More specifically, it has been found that the metal subhalide-alkali metal halide complex mixture, prepared as described below, may be heated directly under prescribed conditions to produce the desired zirconium metal sponge. The process of the invention is carried out by heating the complex mixture at a temperature of about 500° to 700° C., and a pressure of about 0.01 to 100 mm. Hg, preferably about 0.1 to 10.0 mm. Hg. Though the exact nature of the reaction is not understood at this time, it is believed that the aforementioned complexes disproportionate under the influence of the high temperature to give a mixture of the desired metal with metal tetrahalide and alkali metal halide as by-products. During the course of the reaction, the more volatile metal tetrahalide is volatilized and recovered overhead. The reaction is maintained at this temperature for about 1 to 10 hours or until the evolution of metal tetrahalide has substantially ceased.

After the reaction has been completed and the metal tetrahalide volatilized, the remaining reaction products, i.e. the reduced metal and the alkali metal halides, may be further treated in a number of ways to recover the desired metal sponge. One method of operation comprises continuing the heating under vacuum until a temperature of about 700° to 1000° C. is reached. At this temperature the alkali metal halide will volatilize and is recovered overhead. In general, this treatment at elevated temperatures will take about 1 to 10 hours, though it will be understood that heating need only be carried out until substantially all of the alkali metal halide is volatilized. Another method of separating the alkali metal halide from the reduced metal comprises heating the disproportionated reaction mixture, following the volatilization of the metal tetrahalide, at a temperature

2

of about 800° to 1000° C. under atmospheric pressure for about 10 to 20 hours to melt the alkali metal halide and to permit the reduced metal to agglomerate. After sintering, the alkali metal halide can either be distilled off under a vacuum of about 0.1 to 10 microns or leached using conventional techniques such as washing with mineral acid and/or water. It will be understood, that the reaction may be carried out by gradually heating the reaction mixture through the temperature ranges set

10 forth above.

The process of this invention readily lends itself to a continuous operation as well as a batch-type operation. It will be further understood, that metallic impurities present in the crude feed mixtures in the form of their halides also will be separated from the reduced metals in the course of carrying out the process as described above.

As noted above, the feed utilized in the process of the invention comprises the reaction product mixture obtained by partially reducing a metal tetrahalide with an alkali metal. For the purpose of a more complete description, a process using zirconium tetrachloride as the metal halide and metallic sodium as the alkali metal reducing agent will be set forth. Zirconium tetrachloride is passed with metallic sodium into an agitated bed of sodium chloride, which may contain some reduced zirconium chloride or metal from a previous operation, under an inert gas, e.g. argon, atmosphere. The amount of sodium employed will be less than the stoichiometric amount required to completely reduce the zirconium tetrachloride to zirconium metal. Preferably, the amount of sodium employed will constitute about 25 to 50% of the stoichiometric amount. The reaction is carried out at a temperature above the melting point of sodium but below the melting point of the sodium chloride, more specifically at about 150° to 400° C., and preferably about 150° to 200° C. The bed, containing the reaction mixture as well as the reaction products, is maintained in a state of agitation by vigorous mechanical stirring or inert gas fluidization. After the reaction has been completed, a free flowing, finely divided solid dry reaction product mixture is recovered from the reaction vessel.

In accordance with the process described above, feed useful for the present metal manufacture method is prepared, for example, by reacting 49.5 parts of zirconium tetrachloride vapor with 9.75 parts of sodium, this amount of sodium being sufficient for about 50% partial reduction of the zirconium tetrachloride, in a bed of finely divided sodium chloride and zirconium subchlorides at a temperature ranging from about 265° to 575° C. The reaction is carried out in a continuous manner, and the finely divided, free flowing solid reaction product removed continuously from the reactor by means of a screw conveyor. The exact nature of the reaction product mixture is difficult to determine, though it has been established that free zirconium and sodium chloride are not present. However, the reaction products do conform to the empirical formula  $M_aZrX_b$ , wherein M corresponds to the alkali metal employed as the reducing agent and X is the particular halogen used. In accordance with the preferred method of carrying out the invention the atomic ratio of  $a:b$  is about 1:4 to 2:4. Since these reaction products have not been definitely proven to be chemical compounds as contrasted with mixtures, they will be referred to throughout this specification as chemical complexes or compositions.

Though only metallic sodium has been described above as the reducing agent, it will be understood other alkali metals such as lithium, potassium, rubidium and cesium may also be employed. In addition to chlorine as the preferred halogen, bromine and iodine may be effectively utilized. It should also be noted that in place of zirco-

nium, multivalent metals such as titanium, niobium, and molybdenum may be employed. Other multivalent metals may, of course, be employed, provided the metal has a lower but intermediate valence. In this case, the substance employed as the feed material will have an empirical formula corresponding to  $M_aRX_b$ , wherein R is the multivalent metal.

The invention will be further understood by reference to the following illustrative examples.

#### EXAMPLE I

A charge of 8.9 grams of  $Na_2ZrCl_4$  (obtained as the 50% reduction product by reacting  $ZrCl_4$  with metallic sodium) was placed in a tantalum boat and heated to the successively higher temperature tabulated below until only zirconium metal remained as the residue. The by-product  $ZrCl_4$  and  $NaCl$  were collected separately in the cooler parts of the glass tube protruding from the muffle furnace. The more volatile  $ZrCl_4$  was collected at a greater distance from the furnace. The  $NaCl$  was distilled off at pressures in the range of about 0.1 to 10 microns Hg. The results were as follows:

Table I

| Fraction                 | Temp.,<br>°C. | Actual<br>Weight,<br>g. | Theoretical<br>Weight,<br>g. |
|--------------------------|---------------|-------------------------|------------------------------|
| A <sup>1</sup>           | 500-700       | 3.298                   | 3.73                         |
| B <sup>2</sup>           | 700-940       | 3.890                   | 3.73                         |
| C <sup>3</sup> (Residue) |               | 1.757                   | 1.46                         |
| Total                    |               | 8.945                   | 8.92                         |

<sup>1</sup> Substantially  $ZrCl_4$ .

<sup>2</sup> Substantially  $NaCl$ —a Na analysis 34.6% as against 39.4% for theoretical Na in  $NaCl$  (i.e. some  $ZrCl_4$  was present in Fraction B).

<sup>3</sup> Sponge Zr metal.

The discrepancy between the actual and calculated analysis probably arises from the fact that the feed material may vary somewhat from the 50% reduction point. The feed powder may, for example, vary between about 45 and 55% reduction.

#### EXAMPLE II

A charge of about 8.69 grams of 50% reduced  $ZrCl_4$  corresponding to the empirical formula  $Na_2ZrCl_4$  was placed in a tantalum boat and heated under vacuum as in Example I. The  $ZrCl_4$  by-product was condensed farther away from the furnace than the  $NaCl$ , which volatilized later at the higher temperatures by heating for two hours. The results are set forth below:

Table II

| Fraction    | Temp.,<br>°C. | Weight,<br>g. | Remarks                      |
|-------------|---------------|---------------|------------------------------|
| A           | 500-700       | 3.29          | $ZrCl$ contg. 0.25% $NaCl$ . |
| B           | 800-960       | 3.45          | $NaCl$ (36.5% Na).           |
| C (Residue) |               | 1.95          | Sponge Zr Metal (0.114% Cl). |
| Total       |               | 8.69          |                              |

The zirconium sponge produced above had a very open structure. It should be noted that the sponge had a very low chlorine content which is within the A.E.C. specification of 0.15% Cl.

#### EXAMPLE III

A charge of about 10 grams of the approximately 50% reduced  $ZrCl_4$  reaction product mixture was heated under vacuum as set forth in Examples I and II with the excep-

tion that  $NaCl$  volatilization at 0.1 to 10 microns Hg pressure was carried out at a temperature of 900° to 1000° C. for 5 hours. Results are as follows:

Table III

| Fraction    | Temp.,<br>°C. | Weight,<br>g. | Remarks                   |
|-------------|---------------|---------------|---------------------------|
| A           | 600-700       | 3.82          | $ZrCl_4$ (0.43% $NaCl$ ). |
| B           | 900-1,000     | 4.06          |                           |
| C (Residue) |               | 1.89          | Sponge Zr (0.171% Cl).    |
| Total       |               | 9.77          |                           |

It should be noted from the above data that the increased distillation time over that employed in Example II failed to give a zirconium product having a lower chloride ion content. This possibly results from the fact that even with a very open structure the zirconium metal has a residual amount of chloride ion "locked in" which resists removal by vacuum distillation.

It will be apparent that the zirconium tetrachloride and sodium chloride by-products of the invention may readily be employed to advantage in the reduction stage and that this constitutes an additional and significant advantage over prior art processes.

It will be further understood that the reactants and operating conditions set forth in the foregoing specific embodiments may be varied within the limits indicated in the more general description of the invention.

What is claimed is:

1. A process for preparing a multivalent metal selected from the group consisting of zirconium, titanium, niobium, and molybdenum, which consists of (a) reacting a higher valent halide of said metal with about 25 to 50% of the stoichiometric amount of an alkali metal required to completely reduce the higher valent metal halide to metal in an agitated bed of alkali metal halide to obtain a finely divided reaction product corresponding to the empirical formula  $M_aRX_b$ , wherein M is the alkali metal, R is the multivalent metal, X is a halogen selected from the group consisting of chlorine, bromine and iodine, and the ratio of a to b is within the range of about 1:4 to 2:4, (b) heating said finely divided reaction product at a temperature of about 500° to 700° C. to disintegrate said product and to obtain a reaction product mixture comprising said multivalent metal, a higher valent halide of said metal and alkali metal halide, (c) heating said reaction product mixture at a temperature of about 800° to 1000° C. to agglomerate said multivalent metal product, and (d) recovering said agglomerated multivalent metal.

2. The process of claim 1 wherein said multivalent metal is zirconium.

3. The process of claim 1 wherein said alkali metal is sodium.

4. The process of claim 1 wherein said halogen is chlorine.

5. The process of claim 1 wherein the agglomerated multivalent metal is recovered from by-product alkali metal halide by leaching.

6. A process for preparing zirconium metal which consists of (a) reacting zirconium tetrachloride with about 25 to 50% of the stoichiometric amount of an alkali metal required to completely reduce the zirconium tetrachloride to zirconium metal in an agitated bed of alkali metal halide to obtain a finely divided reaction product corresponding to the empirical formula  $M_aZrX_b$ , wherein M is the alkali metal, X is a halogen selected from the group consisting of chlorine, bromine and iodine, and the ratio of a to b is within the range of about 1:4 to 2:4,

(b) heating said finely divided reaction product at a temperature of about 500° to 700° C. to disintegrate

said product and to obtain a reaction product mixture comprising zirconium metal, zirconium tetrahalide and alkali metal halide, and volatilizing said zirconium tetrahalide, (c) heating the remaining reaction product mixture at a temperature of about 800° to 1000° C. under 5 vacuum to agglomerate said zirconium metal and to volatilize said alkali metal halide, and (d) recovering said agglomerated zirconium metal.

7. The process of claim 6 wherein said alkali metal is sodium.

## References Cited in the file of this patent

## UNITED STATES PATENTS

|           |           |               |
|-----------|-----------|---------------|
| 2,707,149 | McKinley  | Apr. 26, 1955 |
| 2,824,799 | Hansley   | Feb. 25, 1958 |
| 2,830,888 | Wade      | Apr. 15, 1958 |
| 2,835,568 | Kingsbury | May 20, 1958  |

## FOREIGN PATENTS

|         |               |               |
|---------|---------------|---------------|
| 717,930 | Great Britain | Nov. 3, 1954  |
| 720,517 | Great Britain | Dec. 22, 1954 |